# EUROPEAN PATENT SPECIFICATION

(11) **EP 4 111 888 B1**
(45) Date of publication and mention of the grant of the patent: **11.09.2024**
(21) Application number: 21761685.3
(22) Date of filing: 07.02.2021
(51) Int. Cl.: A24F 40/46, A24F 40/70, A24F 40/10

(54) **ELECTRONIC ATOMIZATION DEVICE, ATOMIZATION ASSEMBLY, ATOMIZATION ELEMENT AND MANUFACTURING METHOD THEREFOR**
ELEKTRONISCHE ZERSTÄUBUNGSVORRICHTUNG, ZERSTÄUBUNGSANORDNUNG, ZERSTÄUBUNGSELEMENT UND HERSTELLUNGSVERFAHREN DAFÜR
DISPOSITIF D'ATOMISATION ÉLECTRONIQUE, ENSEMBLE D'ATOMISATION, ÉLÉMENT D'ATOMISATION ET PROCÉDÉ DE FABRICATION ASSOCIÉ

(30) Priority: 27.02.2020 CN 202010123152
(43) Date of publication of application: 04.01.2023
(73) Proprietor: Shenzhen Smoore Technology Limited, Shenzhen, Guangdong 518102 (CN)
(72) Inventor: LV, Hongxia, Shenzhen, Guangdong 518102 (CN); JIANG, Zhenlong, Shenzhen, Guangdong 518102 (CN); LI, Pei, Shenzhen, Guangdong 518102 (CN)
(74) Representative: Herrero & Asociados, S.L.
(86) International application number: PCT/CN2021/075810
(87) International publication number: WO 2021/169782

(56) References cited:
- WO-A1-2019/220372
- CN-A- 105 394 816
- CN-A- 106 579 564
- CN-A- 109 414 078
- CN-A- 109 414 078
- CN-A- 109 761 640
- CN-A- 109 875 123
- CN-A- 110 447 959
- CN-A- 111 387 555
- CN-U- 205 337 599
- CN-U- 209 788 491
- GB-A- 2 561 959
- US-A1- 2017 224 021
- US-A1- 2018 007 741
- US-A1- 2021 161 207
- LI, SHOUZE ET AL.: "15. Resistivity of Conductors", COLLECTION OF PHYSICS QUESTIONS, 31 December 1992 (1992-12-31), CN, pages 448, XP009529975, ISBN: 978-7-04-004284-9

## Description

### TECHNICAL FIELD

The present disclosure relates to the field of atomization technology, and in particular, to an electronic atomization device, an atomization assembly, an atomization element, and a method for making the same.

### BACKGROUND

As more attention is paid to the health of human bodies, people are aware of harm of tobacco to the bodies. Therefore, an electronic atomization device is made. The electronic atomization device has an appearance and taste similar to the cigarette, but generally does not include tar, suspended particles, and other harmful ingredients in the cigarette, which greatly reduces harm to a user's body. Therefore, the electronic atomization device is generally used as a substitute for the cigarette and used for giving up smoking.

The electronic atomization device generally includes an atomization assembly and a power supply assembly. A heating element of the atomization assembly of the electronic atomization device currently on the market includes a spring-shaped heating wire. In a producing process of the heating element, a linear heating wire is wound around a fixed shaft; and when the heating wire is powered on, an aerosol-generating material stored on the storage medium is adsorbed onto the fixed shaft and then are atomized by the heating of the heating wire. Another heating element includes a nested combination of a ceramic and a heating wire, but the atomization efficiency is less and aerosol-generating material is leakage to occur. The technology related to the heating element further includes producing a thin-film heating element on a porous ceramic substrate. However, the thin-film heating element has a poor stability of the resistance value and a short service life.

US 2021/0161207 A1 discloses an electronic cigarette, an atomization assembly and an atomization component for the same.The atomization component comprises a porous base, a first film, and a second film. The porous base material comprises an atomization surface. The first film and the second film are sequentially formed on the atomization surface. At least one of the first film or the second film is used for generating heat when charged, so as to heat and atomize an e-liquid on the atomization surface.

US 2018/007741 A1 discloses a heater element, device provided therewith and method for manufacturing such heater element. The heater element comprises a heater of a resistance heating metal that is provided in, at or close to a fluid path configured for heating fluid, wherein the heater comprises a conductor that is provided with a porous ceramic layer. In embodiments, the ceramic layer is provided on or at the conductor with plasma electrolytic oxidation. The ceramic layer has a thickness in the range of 5-300 µm.

US 2017/224021 A1 discloses a forming method for a heating element of an electronic cigarette and a manufacturing method for an atomization assembly, the forming method comprises coiling a heating wire into a heating coil, dividing the heating coil into sections including a plurality of heating sections and connecting sections; providing a deposition preventing layer on an external surface of the heating section; electroplating the heating coil, coating outer peripheral faces of all of the connecting sections of the heating coil with coatings having an electrical resistivity lower than that of the heating wire; removing the deposition preventing layer; and cutting the heating coil electroplated. The present application makes the manufacturing process of the heating element and the atomization assembly continues automatically, the production efficiency is improved, the resistance of the heating element or atomization assembly manufactured is more stable, and the product quality is higher.

### SUMMARY

The present disclosure provides an electronic atomization device, an atomization assembly, an atomization element, and a method for making the atomization element, to overcome the problem that a resistance value of a conductive layer increases excessively fast.

In order to overcome the aforementioned technical problem, a first technical solution provided in the present invention, as defined in claim 1, is an atomization element of an electronic atomization device, the atomization element includes: a porous substrate and a heating layer, the porous substrate includes an atomization surface, and the heating layer covers the atomization surface, the heating layer includes a conductive layer and a stabilizing layer, the conductive layer covers the atomization surface, and the stabilizing layer covers a surface of the conductive layer far away from the porous substrate; and a resistivity of the stabilizing layer is higher than a resistivity of the conductive layer, and oxidation resistance of the stabilizing layer is lower than oxidation resistance of the conductive layer.

Furthermore, a material of the stabilizing layer is selected from the group consisting of an aluminum, a zinc, a tin, a magnesium and a titanium; and a material of the conductive layer is selected from the group consisting of a titanium, a zirconium, a niobium, a tantalum and a 316 stainless steel.

Furthermore, the material of the stabilizing layer is the aluminum; and the material of the conductive layer is a Ti-Zr alloy.

Furthermore, a thickness of the heating layer in the range of 1.5 µm to 5 µm, a thickness of the stabilizing layer in the range of 0.5 µm to 2 µm, and a thickness of the conductive layer in the range of 2 µm to 3 µm.

Furthermore, the atomization element further includes: a first electrode and a second electrode located on the stabilizing layer far away from the porous substrate, wherein a part of the stabilizing layer is covered by the first electrode and the second electrode.

Furthermore, materials of the first electrode and the second electrode are silver.

In order to overcome the aforementioned technical problem, a second technical solution provided in the present disclosure is an atomization assembly of an electronic atomization device, the atomization assembly includes: a liquid storage chamber, configured to store an aerosol-generating material and the atomization element is the atomization element according to any one of the aforementioned, the aerosol-generating material in the liquid storage chamber is able to be transferred to the atomization surface.

In order to overcome the aforementioned technical problem, a third technical solution provided in the present disclosure is an electronic atomization device, includes: a power supply assembly and the atomization assembly according to the aforementioned, the power supply assembly is electrically connected to the atomization assembly to supply power to the atomization element of the atomization assembly.

In order to overcome the aforementioned technical problem, a further technical solution provided in the present invention, as defined in claim 9, is a method for making an atomization element of an electronic atomization device, includes: providing a porous substrate, the porous substrate includes an atomization surface; disposing a conductive layer on the atomization surface of the porous substrate; and disposing a stabilizing layer on a surface of the conductive layer far away from the porous substrate, a resistivity of the stabilizing layer is higher than a resistivity of the conductive layer, and oxidation resistance of the stabilizing layer is lower than oxidation resistance of the conductive layer.

Furthermore, the step of disposing a conductive layer on the atomization surface of the porous substrate includes: disposing the conductive layer on the atomization surface of the porous substrate by adopting a direct-current sputtering deposition process or a magnetron sputtering deposition process; and/or the step of disposing a stabilizing layer on a surface of the conductive layer far away from the porous substrate includes: forming the stabilizing layer on one side of the conductive layer far away from the porous substrate by adopting the direct-current sputtering deposition process or the magnetron sputtering deposition process.

Furthermore, the method further includes: disposing a first electrode and a second electrode on one side of the stabilizing layer far away from the porous substrate and covering a part of the stabilizing layer in a screen-printing manner, and taking a process of low-temperature sintering on the first electrode and the second electrode.

Furthermore, a total thickness of the stabilizing layer and the conductive layer in the range of 1.5 µm to 5 µm, a thickness of the stabilizing layer in the range of 0.5 µm to 2 µm, and a thickness of the conductive layer in the range of 2 µm to 3 µm; and/or a material of the stabilizing layer is selected from the group consisting of an aluminum, a zinc, a tin, a magnesium and a titanium; and a material of the conductive layer is selected from the group consisting of a titanium, a zirconium, a niobium, a tantalum and a 316 stainless steel.

Furthermore, the material of the stabilizing layer is the aluminum; and the material of the conductive layer is a Ti-Zr alloy.

Furthermore, the method further comprising: disposing a first electrode and a second electrode located on the stabilizing layer far away from the porous substrate, and a part of the stabilizing layer is covered by the first electrode and the second electrode.

Furthermore, materials of the first electrode and the second electrode are silver.

Beneficial effects of the present disclosure are as follows. Different from the related art, in the present disclosure, a conductive layer and a stabilizing layer are formed on an atomization surface of a porous substrate, a resistivity of the stabilizing layer is higher than a resistivity of the conductive layer, and oxidation resistance of the stabilizing layer is lower than oxidation resistance of the conductive layer. In the present disclosure, a resistance value of the conductive layer is relatively stable during heating, and does not increase excessively fast, thereby overcoming the problem that the resistance value of the conductive layer increases excessively fast, and bringing an excellent and stable taste to the user.

### BRIEF DESCRIPTION OF THE DRAWINGS

In order to more clearly illustrate the technical solutions of the embodiments of the present disclosure, the drawings for the description of the embodiment will be described in brief. Obviously, the drawings in the following description are only some of the embodiments of the present disclosure. For a person of ordinary skill in the art, other drawings may be obtained based on the following drawings without any creative work.
FIG. 1 is a three-dimensional schematic structural diagram of an electronic atomization device according to an embodiment of the present disclosure.
FIG. 2 is a schematic structural exploded diagram of an atomization assembly of the electronic atomization device shown in FIG. 1.
FIG. 3 is a schematic cross-sectional diagram of a partial enlargement structure of the atomization assembly shown in FIG. 2.
FIG. 4 is a schematic planar structural diagram of an atomization element according to an embodiment of the present disclosure.
FIG. 5 is a process flow diagram of a first embodiment of a method for making an atomization element according to the present disclosure.
FIG. 6 is a process flow diagram of a second embodiment of a method for making an atomization element according to the present disclosure.

### DETAILED DESCRIPTION

Technical solutions of the embodiments of the present disclosure will be clearly and comprehensively described by referring to the accompanying drawings. Obviously, the embodiments described herein are only a part of, but not all of, the embodiments of the present disclosure.

It should be noted that directional indications if present (such as up, down, left, right, front, back, ......) in the embodiments of the present disclosure are only expressed to explain relative positional relationships and movement between components in a particular attitude (as shown in the drawings). When the particular attitude is changed, the directional indications shall also be changed accordingly.

In addition, when using expressions "first", "second", and the like in the embodiment of the present disclosure, the expressions "first", "second", and the like are utilized for descriptive purposes only, and shall not be interpreted as indicating or implying relative importance or implicitly specifying the number of an indicated technical feature. Therefore, features defined by "first" and "second" may explicitly or implicitly include at least one of the such feature. In addition, technical solutions of various embodiments may be combined with each other, but only on the basis that the technical solutions may be achieved by a person of ordinary skill in the art. When combination of technical solutions appears to be contradictory or unachievable, such combination of technical solutions shall be interpreted as inexistence and excluded from the scope of the present disclosure.

The term "comprising" means "including, but not necessarily limited to"; it specifically indicates open-ended inclusion or membership in a so-described combination, group, series and the like. It should be noted that references to "an" or "one" embodiment in this disclosure are not necessarily to the same embodiment, and such references mean at least one. Unless otherwise defined, all technical and scientific terms used herein have the same meaning as a skilled person in the art would understand. The terminology used in the description of the present disclosure is for the purpose of describing particular embodiments and is not intended to limit the disclosure.

Existing common ceramic heating wires cannot heat evenly, and an aerosol-generating material is leakage occur during atomizing. A heating film of a nitride type has a poor stability and a short heating service life. A heating wire of a noble metal type has high costs, and particles are easy to reunite. In order to reduce an increase in the resistance value, the present disclosure provides a new type electronic atomization device, atomization assembly, atomization element, and a method for making the atomization element, which will be described below with reference to the accompanying drawings and embodiments.

Referring to FIG. 1, the electronic atomization device of the present disclosure includes an atomization assembly 100 and a power supply assembly 200. The power supply assembly 200 is electrically connected to the atomization assembly 100, and supply power to the atomization assembly 100.

In one embodiment, the power supply assembly 200 is detachably connected to the atomization assembly 100, so that any one of the atomization assembly 100 and the power supply assembly 200 can be replaced if they are damaged. In other embodiments, the power supply assembly 200 and the atomization assembly 100 may share a same housing, so that the electronic atomization device can be an integral structure and then the electronic atomization device is more convenient to carry. A specific connection manner of the power supply assembly 200 and the atomization assembly 100 is not limited in the embodiments of the present disclosure.

Referring to FIG. 2 and FIG. 3, the atomization assembly 100 includes a liquid storage chamber 10, a cover 20, an airflow channel 30, and an atomization element 40. The atomization element 40 is disposed inside the cover 20, the cover 20 is configured to deliver the aerosol-generating material in the liquid storage chamber 10 into the atomization element 40, and the airflow channel 30 is in communication with an atomization surface of the atomization element 40 to output an atomized aerosol.

In one embodiment, the cover 20 may include a guiding portion 22, a matching portion 24, and a capacity portion 26 that are connected in that order. The guiding portion 22 is provided with a liquid inlet hole 222 and an air outlet hole 224, the liquid inlet hole 222 is in communication with the liquid storage chamber 10, and the air outlet hole 224 is in communication with the airflow channel 30. A cavity chamber 262 for accommodating the atomization element 40 is formed on the capacity portion 26, and the atomization element 40 is accommodated in the cavity chamber 262. The matching portion 24 is configured to communicate the guiding portion 22 with the capacity portion 26, to deliver the aerosol-generating material in the liquid inlet hole 222 to the atomization element 40.

The atomization element 40 is configured to atomize the delivered the aerosol-generating material into aerosol by heating. The air outlet hole 224 is in communication with the atomization surface of the atomization element 40, the aerosol-generating material is heated on the atomization surface and atomized into the aerosol, and the aerosol is delivered through the airflow channel 30 from the air outlet hole 224.

In one embodiment, referring to FIG. 2 and FIG. 3, the cover 20 is an integrally-formed component. For example, the liquid inlet hole 222 and the air outlet hole 224 are separately provided on an end surface of the cover 20 close to the liquid storage chamber 10, and the cavity chamber 262 is formed on an end surface of the capacity portion 26 far away from the liquid storage chamber 10; and finally, a through hole communicated the liquid inlet hole 222 with the cavity chamber 262 is provided on the matching portion 24. Certainly, the guiding portion 22, the matching portion 24, and the capacity portion 26 may alternatively be made on the cover 20 in other machining sequences or manners. That will not be specifically limited herein.

Since the guiding portion 22, the matching portion 24, and the capacity portion 26 are integrally formed structure, the number of elements of the atomization assembly 100 can be reduced, so that a mounting of the atomization assembly 100 is more convenient and the sealing performance is better.

FIG. 4 is a schematic structural diagram of an embodiment of an atomization element of an electronic atomization device according to the present disclosure. The atomization element 40 includes a porous substrate 42 and a heating layer. The heating layer includes a conductive layer 44 and a stabilizing layer 46. The porous substrate 42 includes the atomization surface 422, and the conductive layer 44 and the stabilizing layer 46 are formed on the atomization surface 422 in that order. The aerosol-generating material in the liquid storage chamber 10 is delivered to the porous substrate 42 through the cover 20 and is further delivered onto the atomization surface 422 by the porous substrate 42. Therefore, the aerosol-generating material on the atomization surface 422 may be heated when the conductive layer 44 and/or the stabilizing layer 46 is powered on to generate heat, thereby atomizing the aerosol-generating material into aerosol.

The porous substrate 42 is made of a material with a porous structure, and to be specific, the material may be a porous ceramic, a porous glass, a porous plastic, a porous metal etc. The material of the porous substrate 42 is not specifically limited in present disclosure. In one embodiment, the porous substrate 42 may be made of a material having relatively low temperature resistance, for example, the porous plastic. In another embodiment, the porous substrate 42 may be made of a conductive material with a conductive function, for example, the porous metal.

The porous ceramic has stable chemical properties, and does not chemically react with an aerosol-generating material. The porous ceramic has a high temperature resistance and does not deform due to an excessively high heating temperature. The porous ceramic is an insulator, and is not electrically connected to the conductive layer 44 formed on the porous ceramic to cause a short circuit; and the porous ceramic has advantages of easy manufacturing and low cost. Therefore, in the embodiment, the porous ceramic is selected to make the porous substrate 42.

In an embodiment, a porosity of the porous ceramic may in the range of 30% to 70%. The porosity refers to a ratio of a total volume of tiny pores in a porous medium to a total volume of the porous medium. The size of the porosity may be adjusted according to ingredients of the aerosol-generating material. For example, a relatively high porosity is selected when a viscosity of the aerosol-generating material is relatively large, so as to ensure delivery efficiency of the aerosol-generating material.

In another embodiment, the porosity of the porous ceramic may in the range of 50% to 60%. The porosity of the porous ceramic is controlled in the range of 50% to 60%, on the one hand, the delivery efficiency of the porous ceramic can be ensured, and dry burning caused by poor circulation of the aerosol-generating material is avoided, thereby the atomizing effect is improved. On the other hand, the case that the aerosol-generating material is delivered too fast by the porous ceramic, making it difficult to keep the aerosol-generating material and causing a greatly increased probability of aerosol-generating material leakage can be avoided.

Further, in one embodiment, the conductive layer 44 and the stabilizing layer 46 are both porous films. The conductive layer 44 may be disposed on the atomization surface 422 of the porous substrate 42 by adopting a direct-current sputtering deposition process or a magnetron sputtering deposition process. The stabilizing layer 46 may be formed on one side of the conductive layer 44 far away from the porous substrate 42 by adopting the direct-current sputtering deposition process or the magnetron sputtering deposition process.

Further, the atomization element further includes a first electrode 47 and a second electrode 48 located on the stabilizing layer 46 far away from the porous substrate 42 and cover a part of the stabilizing layer 46 in present disclosure.

In one embodiment, a resistivity of the stabilizing layer 46 is higher than a resistivity of the conductive layer 44, and oxidation resistance of the stabilizing layer 46 is lower than oxidation resistance of the conductive layer 44. In a specific embodiment, a material of the stabilizing layer 46 is selected from the group consisting of an aluminum, a zinc, a tin, a magnesium and a titanium. A material of the conductive layer 44 is selected from the group consisting of a titanium, a zirconium, a niobium, a tantalum and a 316 stainless steel. Materials of the first electrode 47 and the second electrode 48 are silver. In an embodiment, the material of the stabilizing layer 46 is aluminum. The material of the conductive layer 44 is a Ti-Zr alloy.

The features of the titanium and zirconium are as follows.
(1) Titanium and zirconium are both metals having good biocompatibility, and especially, titanium is a biophile metal element having a higher safety.
(2) Titanium and zirconium have a larger resistivities among metal materials. In a normal temperature, a Ti-Zr alloy has a resistivity three times than an original resistivity after alloying according to a specific proportion, which is more suitable for being used as a heating film material.
(3) Titanium and zirconium have small thermal expansion coefficients, and the Ti-Zr alloy has a smaller thermal expansion coefficient after alloying, and has a better thermal matching with the porous ceramic. After titanium is alloyed with zirconium according to a specific proportion, the Ti-Zr alloy has a lower melting point, and the film-forming property of magnetron sputtering coating is better.
(4) After coating of a metal, it can be seen by electron microscope analysis that microscopic particles of the metal are spherical, and the particles are crowded together to form a microscopic morphology similar to cauliflower; while it can be seen by electron microscope analysis that microscopic particles of a film formed by the Ti-Zr alloy are sheet-shaped, and some grain boundaries between particles disappear, to provide a better continuity.
(5) Titanium and zirconium both have well plasticity and elongation rate, and the Ti-Zr alloy film has a better resistance to thermal cycling and current surge.
(6) Titanium is usually used as a stress buffer layer of metals and ceramics, and an activation element of ceramic metallization, and titanium can be reacted with a ceramic surface to form a relatively strong chemical bond, which may improve the adhesion of the film.

Furthermore, since the titanium-zirconium in a Ti-Zr alloy film has poor stability in the air at high temperature, zirconium can easily absorb hydrogen gas, nitrogen gas, and oxygen gas, and the Ti-Zr alloy has better inspiratory after alloying, thus the stabilizing layer 46 is needed to cover the conductive layer 44 after the conductive layer 44 is made, and the material of the stabilizing layer 46 is aluminum.

In an embodiment, after the stabilizing layer 46 (an aluminum layer) is made, the first electrode 47 and the second electrode 48 are made in a screen-printing manner, and taking a process of low-temperature sintering on the first electrode 47 and the second electrode 48. The first electrode 47 and the second electrode 48 cover a part of the stabilizing layer 46. On the one hand, when the first electrode 47 and the second electrode 48 are formed in a low-temperature sintering manner, a relatively dense aluminum oxide layer is formed on a surface of the stabilizing layer 46, so that the conductive layer 44 can be isolated from air, thereby a resistance value of the conductive layer 44 can be prevented from being increased, to overcome the problem of the suction taste being changed and suction instability due to an increase in a resistance value of the heating layer. On the other hand, when the first electrode 47 and the second electrode 48 are made in the low-temperature sintering manner, as the first electrode 47 and the second electrode 48 are sintered, thereby a region of the stabilizing layer 46 covered by the first electrode 47 and the second electrode 48 can be prevented from being oxidized, and contact resistance can be avoided.

Since a melting point of aluminum is 660°C and a melting point of aluminum oxide is 2054°C, the stabilizing layer 46 can maintain the stability and a particle reuniting is not easy to occur during atomizing. Compared with the case that particle reuniting is easy to occur in a noble metal protective layer such as Au/Ag during atomizing and causing failure of a heating element, selecting aluminum as the material of the stabilizing layer 46 can overcome this issue. On the other hand, aluminum oxide has same main ingredients as the ceramic, which has a low thermal expansion coefficient, and has smaller deformation during current surge.

The stabilizing layer 46 is made of aluminum, and the overall resistivity is larger than that of a noble metal. A resistivity of the noble metal in the range of 0.8 ohms to 1.2 ohms, and the resistivity of aluminum has a minimum value of about 1 ohm through parameter adjustment and substantially in the range of 1.5 ohms to 3 ohms. In addition, resistivities of the conductive layer 44 and the stabilizing layer 46 are relatively close by adopting the aforementioned method, which can prevent a current of one of the layers from being excessively large. Theoretically, a thermal expansion coefficient of the noble metal gold is 14.2, but a thermal expansion coefficient of aluminum oxide formed after aluminum is sintered is about half of gold, namely, 7.1. Therefore, a deformation rate of the conductive layer is lower during sucking, and the stability is improved.

In a specific embodiment, a thickness of the heating layer is in the range of 1.5 µm to 5 µm; the heating layer includes the conductive layer 44 and the stabilizing layer 46. For example, the thickness of the conductive layer 44 is in the range of 2 µm to 3 µm, and the thickness of the stabilizing layer 46 is in the range of 0.5 µm to 2 µm.

In summary, in the embodiments of the present disclosure, the material of the conductive layer 44 is selected from the group consisting of the titanium, the zirconium, the niobium, the tantalum and the 316 stainless steel, and the material of the stabilizing layer 46 is selected from the group consisting of the aluminum, the zinc, the tin, the magnesium, and the titanium. Furthermore, the first electrode 47 and the second electrode 48 are made in the low-temperature sintering manner, so as to the service life of the heating element is prolonged, and the increase of the resistance value is reduced, and the contact resistance is avoided.

FIG. 5 is a schematic flow diagram of a first embodiment of a method for making an atomization element of an electronic atomization device according to the present disclosure. The method includes the following steps.

Step S51: providing a porous substrate; the porous substrate including an atomization surface.

The porous substrate is made of a material with a porous structure, and to be specific, the material may be a porous ceramic, a porous glass, a porous plastic, a porous metal etc. The material of the porous substrate is not specifically limited in present disclosure. In one embodiment, the porous substrate may be made of a material having relatively low temperature resistance, for example, the porous plastic. In another embodiment, the porous substrate may be made of a conductive material with a conductive function, for example, the porous metal. The porous substrate includes the atomization surface.

Step S52: disposing a conductive layer on the atomization surface of the porous substrate.

The conductive layer is formed on the atomization surface of the porous substrate by adopting a magnetron sputtering deposition process or a direct-current sputtering deposition process. For example, a material of the conductive layer is selected from the group consisting of the titanium, the zirconium, the niobium, the tantalum and the 316 stainless steel. Take the conductive layer which is disposed by adopting the direct-current sputtering deposition process for example, a specific method is as follows: A vacuum degree is kept in a range of 8×10-4 Pa to 2×10-3 Pa; a power is kept in a range of 1500 W to 2500 W, and a time is kept in a range of 70 min to 110 min; and a pressure is kept in a range of 0.3 Pa to 0.8 Pa, a temperature is kept in a range of a room temperature to 300°C, and a particle diameter is kept approximately in a range of 200 nm to 400 nm.

Step S53: disposing a stabilizing layer on a surface of the conductive layer far away from the porous substrate.

The stabilizing layer is disposed on the surface of the conductive layer far away from the porous substrate by adopting the magnetron sputtering deposition process or the direct-current sputtering deposition process. For example, the material of the stabilizing layer is selected from the group consisting of the aluminum, the zinc, the tin, the magnesium, and the titanium. Take the stabilizing layer which is disposed by adopting the direct-current sputtering deposition process for example, a specific method is as follows: A time is in the range of 40 min to 60 min, a power is in the range of 500 W to 1500 W, a pressure is in the range of 1 Pa to 1.5 Pa, and a temperature is in the range of a room temperature to 300°C. A particle diameter ranges approximately from 100 nm to 200 nm.

In one embodiment, the conductive layer and the stabilizing layer are formed on the atomization surface in that order. An aerosol-generating material in the liquid storage chamber is delivered to the porous substrate through the cover and is further delivered onto the atomization surface by the porous substrate. Therefore, the aerosol-generating material on the atomization surface may be heated when the conductive layer and/or the stabilizing layer is powered on to generate heat, thereby atomizing the aerosol-generating material into aerosol.

In an embodiment, a total thickness of the conductive layer and the stabilizing layer is 1.5 µm; a thickness of the conductive layer is in the range of 2 µm to 3 µm, and a thickness of the stabilizing layer is in the range of 0.5 µm to 2 µm.

In an embodiment, a resistivity of the stabilizing layer is higher than a resistivity of the conductive layer, and oxidation resistance of the stabilizing layer is lower than oxidation resistance of the conductive layer. For example, the material of the stabilizing layer is aluminum, and the material of the conductive layer is a Ti-Zr alloy.

In the present disclosure, the material of the conductive layer is selected from the group consisting of the titanium, the zirconium, the niobium, the tantalum and the 316 stainless steel, and the material of the stabilizing layer is selected from the group consisting of the aluminum, the zinc, the tin, the magnesium, and the titanium. Therefore, the relatively dense aluminum oxide layer can be formed on the surface of the stabilizing layer, so that the conductive layer can be isolated from air, thereby the resistance value of the conductive layer can be reduced, to overcome the problem of the suction taste being changed and suction instability due to the increase in the resistance value of the conductive layer.

FIG. 6 is a schematic flow diagram of a second embodiment of a method for making an atomization element of an electronic atomization device according to the present disclosure.

Step S61, step S62, and step S63 are respectively the same as step S51, step S52, and step S53 in the first embodiment shown in FIG. 5. A difference is, the embodiment further includes step S64: disposing a first electrode and a second electrode cover a part of the stabilizing layer on one side of the stabilizing layer far away from the porous substrate in a screen-printing manner, and taking a process of low-temperature sintering on the first electrode and the second electrode.

For example, materials of the first electrode and the second electrode are silver. The first electrode and the second electrode covering a part of the stabilizing layer are disposed on one side of the stabilizing layer far away from the porous substrate in the screen-printing manner. The first electrode and the second electrode cover a part of the stabilizing layer. Then taking a process of low-temperature sintering on the first electrode and the second electrode. when the first electrode and the second electrode are formed in a low-temperature sintering manner, a relatively dense aluminum oxide layer is formed on a surface of the stabilizing layer, so that the conductive layer can be isolated from air, thereby a resistance value of the conductive layer can be prevented from being increased, to overcome the problem of the suction taste being changed and suction instability due to an increase in a resistance value of the heating layer. On the other hand, when the first electrode and the second electrode are made in the low-temperature sintering manner, as the first electrode and the second electrode are sintered, thereby a region of the stabilizing layer covered by the first electrode and the second electrode can be prevented from being oxidized, and contact resistance can be avoided.

## Claims

1. An atomization element (40) of an electronic atomization device, the atomization element (40) comprising:
a porous substrate (42) and a heating layer, wherein the porous substrate (42) comprises an atomization surface (422), and the heating layer covers the atomization surface (422), wherein
the heating layer comprises an electrically conductive layer (44) and a stabilizing layer (46), the electrically conductive layer (44) covers the atomization surface (422), and the stabilizing layer (46) covers a surface of the
electrically conductive layer (44) which is opposite to the surface which is in contact with the porous substrate (42); and
**characterized by** that, an electrical resistivity of the stabilizing layer (46) is higher than an electrical resistivity of the electrically conductive layer (44), and oxidation resistance of the stabilizing layer (46) is lower than oxidati resistance of the electrically conductive layer (44).

2. The atomization element (40) of claim 1, wherein a material of the stabilizing layer (46) is selected from the group consisting of an aluminum, a zinc, a tin, a magnesium and a titanium; and a material of the electrically conductive layer (44) is selected from the group consisting of a titanium, a zirconium, a niobium, a tantalum and a 316 stainless steel.

3. The atomization element (40) of claim 2, wherein the material of the stabilizing layer (46) is the aluminum; and the material of the electrically conductive layer (44) is a Ti-Zr alloy.

4. The atomization element (40) of claim 1, wherein a thickness of the heating layer in the range of 1.5 µm to 5 µm, wherein
a thickness of the stabilizing layer (46) in the range of 0.5 µm to 2 µm, and a thickness of the
electrically conductive layer (44) in the range of 2 µm to 3 µm.

5. The atomization element (40) of any one of claims 1 to 4, further comprising: a first electrode (47) and a second electrode (48) located on the stabilizing layer (46) which is opposite to the surface which is in contact with the porous substrate (42), wherein a part of the stabilizing layer (46) is covered by the first electrode (47) and the second electrode (48).

6. The atomization element (40) of claim 5, wherein materials of the first electrode (47) and the second electrode (48) are silver.

7. An atomization assembly (100) of an electronic atomization device, the atomization assembly (100) comprising:
a liquid storage chamber (10), configured to store an aerosol-generating material and the atomization element (40) according to any one of claims 1 to 6, wherein the aerosol-generating material in the liquid storage chamber (10) is able to be transferred to the atomization surface (422).

8. An electronic atomization device, comprising:
a power supply assembly (200); and the atomization assembly (100) according to claim 7, wherein the power supply assembly (200) is electrically connected to the atomization assembly (100) to supply power to the atomization element (40) of the atomization assembly (100).

9. A method for making an atomization element (40) of an electronic atomization device, comprising:
providing a porous substrate (42), wherein the porous substrate (42) comprises an atomization surface (422);
disposing an electrically conductive layer (44) on the atomization surface (422) of the porous substrate (42); and
disposing a stabilizing layer (46) on a surface of the electrically conductive layer (44) which is opposite to the surface which is in contact with the porous substrate (42),
**characterized by** that, an electrical resistivity of the stabilizing layer (46) is higher than an electrical resistivity of the
electrically conductive layer (44), and oxidation resistance of the stabilizing layer (46) is lower than oxidation resistance of the electrically conductive layer (44).

10. The method of claim 9, wherein the step of disposing an electrically conductive layer (44) on the atomization surface (422) of the porous substrate (42) comprises:
disposing the electrically conductive layer (44) on the atomization surface (422) of the porous substrate (42) by adopting a direct-current sputtering deposition process or a magnetron sputtering deposition process; and/or
the step of disposing a stabilizing layer (46) on a surface of the electrically conductive layer (44) which is opposite to the surface which is in contact with the porous substrate (42) comprises:
forming the stabilizing layer (46) on one side of the electrically conductive layer (44) which is opposite to the surface which is in contact with the porous substrate (42) by adopting the direct-current sputtering deposition process or the magnetron sputtering deposition process.

11. The method of claim 9, further comprising:
disposing a first electrode (47) and a second electrode (48) on one side of the stabilizing layer (46) which is opposite to the surface which is in contact with the porous substrate (42), and covering a part of the stabilizing layer (46) in a screen-printing manner, and taking a process of low-temperature sintering on the first electrode (47) and the second electrode (48).

12. The method according to any one of claims 9 to 11, wherein a total thickness of the stabilizing layer (46) and the electrically
conductive layer (44) in the range of 1.5 µm to 5 µm, wherein a thickness of the stabilizing layer (46) in the range of 0.5 µm to 2 µm, and a thickness of the electrically conductive layer (44) in the range of 2 µm to 3 µm; and/or
a material of the stabilizing layer (46) is selected from the group consisting of an aluminum, a zinc, a tin, a magnesium and a titanium; and
a material of the electrically conductive layer (44) is selected from the group consisting of a titanium, a zirconium, a niobium, a tantalum and a 316 stainless steel.

13. The method of claim 12, wherein the material of the stabilizing layer (46) is the aluminum; and the material of the electrically conductive layer (44) is a Ti-Zr alloy.

14. The method according to any one of claims 9 to 10, further comprising: disposing a first electrode (47) and a second electrode (48) on the stabilizing layer (46) which is opposite to the surface which is in contact with the porous substrate (42), wherein a part of the stabilizing layer (46) is covered by the first electrode (47) and the second electrode (48).

15. The method of claim 14, wherein materials of the first electrode (47) and the second electrode (48) are silver.

## Patentansprüche

1. Ein Zerstäubungselement (40) einer elektronischen Zerstäubungsvorrichtung, Zerstäubungselement (40), das Folgendes umfasst:
Ein poröses Substrat (42) und eine Heizschicht, wobei das poröse Substrat (42) eine Zerstäubungsfläche (422) umfasst und eine Heizschicht die Zerstäubungsfläche (422) deckt, wobei
die Heizschicht eine elektrisch leitende Schicht (44) und eine Stabilsierungsschicht (46) umfasst, die elektrische leitende Schicht (44) die Zerstäubungsfläche (422) deckt und die Stabilisierungsschicht (46) eine Oberfläche der elektrisch leitenden Schicht (44) deckt, die der Oberfläche gegenüberliegt, die mit dem porösen Substrat (42) im Kontakt steht; und
**dadurch gekennzeichnet, dass** eine elektrische Widerstandsfähigkeit der Stabilisierungsschicht (46) grösser ist als eine elektrische Widerstandsfähigkeit der elektrisch leitenden Schicht (44), eine Oxidationsbeständigkeit der Stabilisierungsschicht (46) geringer ist als als die Oxidationsbeständigkeit der elektrisch leitenden Schicht (44).

2. Das Zerstäubungselement (40) gemäss Anspruch 1, bei dem ein Material der Stabilisierungsschicht (46) ausgewählt wird aus der Gruppe bestehend aus einem Aluminium, einem Zink, einem Zinn, einem Magnesium und einem Titan; und ein Material der eletrisch leitenden Schicht (44) ausgewählt aus der Gruppe bestehend aus einem Titan, Zirkon, Niob, Tantal und 316 rostfreiem Staal

3. Das Zerstäubungselement (40) gemäss Anspruch 2, bei dem das Material der Stabilisierungsschicht (46) das Aluminium ist; und das Material der elektrisch leitenden Schicht (44) eine Ti-Zr-Legierung ist.

4. Das Zerstäubungselement (40) gemäss Anspruch 1, bei dem eine Stärke der Heizschicht im Bereich von 1,5 µm bis 5 µm liegt, wobei eine Stärke der Stabilisierungsschicht (46) im Bereich von 0,5 µm bis 2 µm, und eine Stärke der elektrisch leitenden Schicht (44) im Bereich 2 µm bis 3 µm liegt.

5. Das Zerstäubungselement (40) gemäs irgendeinem der Ansprüche 1 bis 4, das weiter Folgendes umfasst: eine an der Stabilisierungsschicht (46) lokalisierte erste Elektrode (47) und zweite Elektrode (48), Stabilisierungsschicht, die gegenüber der Oberfläche liegt, die im Kontakt mit dem porösen Substrat (42) ist, wobei ein Teil der Stabilisierungsschicht (46) durch die erste Elektrode (47) und zweite Elektrode (46) bedeckt ist.

6. Das Zerstäubungselement (40) gemäss Anspruch 5, bei dem das Material der ersten Elektrode (47) und der zweiten Elektrode (48) Silber ist.

7. Eine Zerstäubungsgruppe (100) einer elektronischen Zerstäubungsvorrichtung, wobei die Zerstäubungsgruppe (100) Folgendes umfasst:
Eine Flüssigkeitsspeicherkammer (100), die konfiguriert ist, um ein Aerosolerzeugungsmaterial und das Zerstäubungselement (40) gemäss irgendeinem der Ansprüche 1 bis 6 zu speichern, wobei das Aerosolerzeugungsmaterial in der Flüssigkeitsspeicherkammer (10) zur Zerstäubungsfläche (422) gefördert werden kann.

8. Eine elektronische Zerstäubungsvorrichtung, die Folgendes umfasst:
Eine Stromversorgungsbaugruppe (200) und die Zerstäubungsgruppe (100) gemäss Anspruch 7, wobei die Stromversorgungsbaugruppe (200) elektrisch an die Zerstäubungsgruppe (100) angeschlossen ist, um das Zerstäubungselement (40) der Zerstäubungsgruppe (100) mit Strom zu versorgen.

9. Eine Methode für die Herstellung eines Zerstäubungselements (40) einer elektronischen Zerstäubungsvorrichtung, die Folgendes umfasst:
Bereitstellung eines porösen Substrats (42), wobei das poröse Substrat (42) eine Zerstäubungsoberfläche (422) umfasst;
Anordnen einer elektrisch leitenden Schicht (44) auf der Zerstäubungsoberfläche (422) des porösen Substrats (42);
und
Anordnen einer Stabilisierungsschicht (46) auf einer Oberfläche der elektrisch leitenden Schicht (44), Oberfläche, die derjenigen gegenüberliegt, die im Kontakt mit dem porösen Substrat (42) steht,
**dadurch gekennzeichnet, dass** eine elektrische Widerstandsfähigkeit der Stabilisierungsschicht (46) grösser ist als eine elektrische Widerstandsfähigkeit der elektrisch leitenden Schicht (44), und eine Oxidationsbeständigkeit der Stabilisierungsschicht (46) geringer ist als die Oxidationsbeständigkeit der elektrisch leitenden Schicht (44).

10. Die Methode gemäss Anspruch 9, bei der der Schritt des Anordnens einer elektrisch leitenden Schicht (44) auf der Zerstäubungsoberfläche (422) des porösen Substrats (42) Folgendes umfasst:
Abscheiden der elektrisch leitenden Schicht (44) auf der Zerstäubungsoberfläche (422) des porösen Substrats (42) mittles Anwendung eines Gleichstromssputter-Abscheidungsverfahrens oder eines Magnetronsputter-Abscheidungsverfahrens; und/oder
wobei der Abscheidungsschritt einer Stabilisierungsschicht (46) auf einer Oberfläche der elektrisch leitenden Schicht, die der Oberfläche gegenüberliegt, die im Kontakt steht mit dem porösen Substrat (42), Folgendes umfasst:
das Formen der Stabilisierungsschicht (46) an einer Seite der elektrisch leitenden Schicht (44), die der Oberfläche gegenüberliegt, die im Kontakt steht mit dem porösen Substrat (42), indem das Gleichstromsputter-Abscheidungsverfahren oder das Magnetronsputter-Abscheidungsverfaren angewandt wird.

11. Die Methode gemäss Ansprhc 9, die weiter Folgendes umfasst:
Anordnen einer ersten Elektrode (47) und einer zweiten Elektrode (48) an einer Seite der Stabilisierungsschicht (46), die der Oberfläche gegenüberlliegt, die im Kontakt mit dem porösen Substrat (42) steht, und Bedecken eines Teils der Stabilisierungsschicht (46) mittels einer Siebdruckmethode, und Anwenden eines Verfahrens einer Niedrigtemperatursinterung an der ersten Elektrode (47) und zweiten Elektrode (48).

12. Die Methode gemäss irgendeinem der Ansprüche 9 bis 11, bei der eine Gesamtstärke der Stabilisierungsschicht (46) und der elektrisch leitenden Schicht (4) sich im Bereich von 1,5 µm bis 5 µm befindet, wobei eine Stärke der Stabilisierungsschicht (46) sich im Bereich von 0,5 µm bis 2 µm befindet und eine Stärke der elektrisch leitenden Schicht (44) im Bereich von 2 µm bis 3 µm befindet; und/oder
ein Material der Stabilisierungsschicht (46) ausgewählt wird aus der Gruppe besteehend aus einem Aluminium, einem Zink, einem Zinn, einem Magnesium und einem Titan; und
ein Material der elektrisch leitenden Schicht (44) ausgewählt wird aus der Gruppe bestehend aus einem Titan, einem Zirkon, einem Niob, einem Tantal und einem 316 rostfreien Stahl.

13. Die Methode gemäss Anspruch 12, bei der das Material der Stabilisierungsschicht (46) das Aluminium und das Material der elektrisch leitenden Schicht (44) eine Ti-Zr-Legierung ist.

14. Die Methode gemäss irgendeinem der Ansprüche 9 bis 10, die weiter Folgendes umfasst: Abscheiden einer ersten Elektrode (47) und zweiten Elektrode (48) auf der Stabilisierungsschicht (46), die gegenüber der im Kontakt mit dem porösen Substrat stehenden Oberfläche liegt, wobei ein Teil der Stabilisierungsschicht (46) durch die erste Elektrode (47) und zweite Elektrode (48) bedeckt ist.

15. Die Methode gemäss Anspruch 14, bei der das Material der ersten Elektrode (47) und zweiten Elektrode (48) Silber ist.

## Revendications

1. Un élément d'atomisation (40) d'un dispositif électronique d'atomisation, dans lequel ledit élément d'atomisation (40) comprend :
un substrat poreux (42) et une couche chauffante, où le substrat poreux (42) comprend une surface d'atomisation (422), et la couche chauffante couvre la surface d'atomisation (422), et où
la couche chauffante comprend une couche électriquement conductrice (44) et une couche de stabilisation (46), la couche électriquement conductrice (44) couvre la surface d'atomisation (422), et la couche de stabilisation (46) recouvre une surface de la couche électriquement conductrice (44) opposée à la surface qui est en contact avec le substrat poreux (42) ; et
**caractérisé en ce que** la résistivité électrique de la couche de stabilisation (46) est supérieure à la résistivité électrique de la couche électriquement conductrice (44), et la résistance à l'oxydation de la couche de stabilisation (46) est inférieure à la résistance à l'oxydation de la couche électriquement conductrice (44).

2. L'élément d'atomisation (40) selon la revendication 1, dans lequel un matériau de la couche de stabilisation (46) est choisi dans le groupe constitué par l'aluminium, le zinc, l'étain, le magnésium et le titane ; et un matériau de la couche électriquement conductrice (44) est choisi dans le groupe constitué par le titane, le zirconium, le niobium, le tantale et l'acier inoxydable 316.

3. L'élément d'atomisation (40) selon la revendication 2, dans lequel le matériau constitutif de la couche de stabilisation (46) est l'aluminium et le matériau choisi pour la couche conductrice d'électricité (44) est un alliage Ti-Zr.

4. L'élément d'atomisation (40) selon la revendication 1, dans lequel l'épaisseur de la couche chauffante est comprise entre 1,5 µm et 5 µm, l'épaisseur de la couche de stabilisation (46) est comprise entre 0,5 µm et 2 µm, et l'épaisseur de la couche conductrice d'électricité (44) est comprise entre 2 µm et 3 µm.

5. L'élément d'atomisation (40) selon une quelconque des revendications 1 à 4, comprenant en outre : une première électrode (47) et une deuxième électrode (48) situées sur la couche de stabilisation (46) opposée à la surface qui est en contact avec le substrat poreux (42), une partie de la couche de stabilisation (46) étant recouverte par la première électrode (47) et la deuxième électrode (48).

6. L'élément d'atomisation (40) selon la revendication 5, dans lequel le matériau utilisé pour la première électrode (47) et la seconde électrode (48) est de l'argent.

7. Module d'atomisation (100) d'un dispositif électronique d'atomisation, le module d'atomisation (100) comprenant :
une chambre de stockage de liquide (10), configurée pour stocker un matériau générateur d'aérosol et l'élément d'atomisation (40) selon une quelconque des revendications 1 à 6, dans lequel le matériau générateur d'aérosol contenu dans la chambre de stockage de liquide (10) est capable d'être transféré vers la surface d'atomisation (422).

8. Dispositif électronique d'atomisation comprenant :
un bloc d'alimentation électrique (200) ; et le module d'atomisation (100) selon la revendication 7, dans lequel le bloc d'alimentation électrique (200) est connecté électriquement au module d'atomisation (100) pour alimenter en électricité l'élément d'atomisation (40) du module d'atomisation (100).

9. Procédé de fabrication d'un élément d'atomisation (40) d'un dispositif électronique d'atomisation, comprenant :
fournir un substrat poreux (42), où le substrat poreux (42) comprend une surface d'atomisation (422) ;
déposer une couche électriquement conductrice (44) sur la surface d'atomisation (422) du substrat poreux (42) ;
et
déposer une couche de stabilisation (46) sur une surface de la couche électriquement conductrice (44) opposée à la surface qui est en contact avec le substrat poreux (42),
**caractérisé en ce que** la résistivité électrique de la couche de stabilisation (46) est supérieure à la résistivité électrique de la couche électriquement conductrice (44), et la résistance à l'oxydation de la couche de stabilisation (46) est inférieure à la résistance à l'oxydation de la couche électriquement conductrice (44).

10. Procédé selon la revendication 9, dans lequel l'étape consistant à déposer une couche électriquement conductrice (44) sur la surface d'atomisation (422) du substrat poreux (42) comprend :
déposer la couche électriquement conductrice (44) sur la surface d'atomisation (422) du substrat poreux (42) en adoptant un procédé de dépôt par pulvérisation cathodique à courant continu ou un procédé de dépôt par pulvérisation cathodique à magnétron ; et/ou
l'étape consistant à déposer une couche de stabilisation (46) sur une surface de la couche électriquement conductrice (44) opposée à la surface en contact avec le substrat poreux (42) comprend : la formation de la couche de stabilisation (46) sur un côté de la couche électriquement conductrice (44) opposée à la surface qui est en contact avec le substrat poreux (42, en adoptant le procédé de dépôt par pulvérisation cathodique à courant direct ou le procédé de dépôt par pulvérisation cathodique à magnétron.

11. Le procédé selon la revendication 9, comprenant en outre :
déposer une première électrode (47) et une deuxième électrode (48) sur un côté de la couche de stabilisation (46) opposé à la surface qui est en contact avec le substrat poreux (42), et recouvrir une partie de la couche de stabilisation (46) par un procédé de sérigraphie, et exécuter un traitement de frittage à basse température sur la première électrode (47) et la deuxième électrode (48).

12. Le procédé selon une quelconque des revendications 9 à 11, dans lequel une épaisseur totale de la couche de stabilisation (46) et de la couche électriquement conductrice (44) est comprise entre 1,5 µm et 5 µm, l'épaisseur de la couche de stabilisation (46) étant comprise entre 0,5 µm et 2 µm, et l'épaisseur de la couche électriquement conductrice (44) étant comprise entre 2 µm et 3 µm ; et/ou
un matériau de la couche de stabilisation (46) est choisi parmi le groupe constitué par l'aluminium, le zinc, l'étain, le magnésium et le titane ; et
un matériau de la couche conductrice d'électricité (44) est choisi parmi le groupe constitué par le titane, le zirconium, le niobium, le tantale et l'acier inoxydable 316.

13. Procédé selon la revendication 12, dans lequel le matériau choisi pour la couche de stabilisation (46) est l'aluminium et le matériau choisi pour la couche conductrice d'électricité (44) est un alliage Ti-Zr.

14. Procédé selon une quelconque des revendications 9 à 10, comprenant en outre les étapes suivantes : le dépôt d'une première électrode (47) et d'une deuxième électrode (48) sur la couche de stabilisation (46) opposée à la surface qui est en contact avec le substrat poreux (42), une partie de la couche de stabilisation (46) étant recouverte par la première électrode (47) et la deuxième électrode (48).

15. Procédé selon la revendication 14, dans lequel le matériau utilisé pour la première électrode (47) et la seconde électrode (48) est de l'argent.
